

## UNITED STATES PATENT OFFICE

SIGISMUND FUCHS, OF HÖCHST-ON-THE-MAIN, GERMANY, ASSIGNOR TO FIRM OF DURAND & HUGUENIN S. A., OF BASEL, SWITZERLAND

## DYEING PROCESS FOR ANIMAL FIBERS

No Drawing. Application filed December 22, 1930, Serial No. 504,928, and in Germany December 22, 1930.

Watersoluble esterlike derivatives (ester-salts) of insoluble dyestuffs containing quinone groups, these latter being in a reduced form and esterified (see for instance U. S. Patent No. 1,448,251), are employed for dyeing, printing etc. by applying such bodies onto a fiber and by developing the colour by acid oxidation. The said ester salts have—like acid dyestuffs—an affinity for the animal fiber. Such an ester salt may be applied from an acid bath to wool, silk etc. and on this latter the dyeing may be developed by acid oxidation (see also U. S. Patent No. 1,575,958).

It has been observed that by this last named method it is often difficult to develop the dyeing in a suitable manner. Over-oxidation of the dyestuff or a too strong yellowing of the fiber (wool) caused by the excess of the oxidizing agents, is very liable to take place, so that dull and loose to light shades are obtained.

It has now been found that this over-oxidation of the dyestuff, respectively the too strong yellowing of the fiber (wool), when the usual oxidizing agents, such as for instance bichromate of potash, are used, can be avoided to a great extent if watersoluble salts of hydrosulphocyanic acid, such as sulphocyanide of ammonia, sulphocyanide of potash, are added to the developing bath.

For carrying out the improved process the ester-salts are brought on to the fiber in the usual way. Subsequently the development is performed in a bath, to which, besides the oxidizing agent and an acid, a sulphocyanide has been added.

It is known, that sulphocyanides are used for dyeing and printing purposes. When dyeing or printing artificial fibers for instance, they may be used as swelling agent. They may further be used as acid forming substance (see U. S. Patent No. 1,779,305).

In the present process, however, wherein development is carried out in a bath, to which besides the oxidizing agent, acid is added, the

sulphocyanides act as buffer substances. They prevent over-oxidation and are themselves probably destroyed by oxidation.

The improved process may be illustrated by the following examples, without limiting it thereto.

## Examples for wool

(I) a. Dyeing.—For 100 kilos of woolen material a dyebath is prepared with 0.2 kg. of ester-salt of leucotetra-bromindigo (40%) and 5 kg. of sulphate of ammonia. Enter at 40° C., raise to the boil in 1/2 hour, boil for 1/2 hour, add acetic acid in order to exhaust the dyebath, boil for a further 1/2 hour and let cool down.

b. Development.—Oxidize in a bath containing 2 kg. of sulphocyanide of ammonia and 1 kg. of bichromate of potash, treat for 1/4 hour at 30° C. After having added slowly 10 gr. of sulphuric acid of 66° Bé. per liter of liquor, heat up to 85° C. in 1/2 hour, treat for 1/2 hour at 85-90° C., rinse, neutralize and rinse again.

(II) a. Dyeing.—For 100 kilos of woolen material a dyebath is prepared with 0.2 kg. of ester-salt of leuco-4:4'-dimethyl-6:6'-dichlorothioindigo and 5 kg. of sulphate of ammonia. Enter at 40° C., raise to the boil in 1/2 hour, boil for 1/2 hour, and add 1 kg. of acetic acid. Dye for further 1/2 hour at the boil until the bath is exhausted.

b. Development.—Prepare a fresh bath containing 1% of sulphocyanide of ammonia and 1.1% of bichromate of potash, treat for 1/4 hour at 30° C. and add 10 gr. of sulphuric acid of 66° Bé. per liter of liquor, heat up to 85° C. in 1/2 hour, maintain at 85-90° C. for 1/2 hour, rinse, neutralize, and rinse again.

(III) a. Dyeing.—For 100 kilos of woolen material a dyebath is prepared with 1 kg. of ester-salt of leuco-3:4:8:9-dibenzpyrene-5:10-quinone and 5 kg. of sulphate of ammonia. Enter at 40° C., raise to the boil in 1/2 hour, boil for 1/2 hour, and add 2 kg. of

acetic acid. Boil for a further  $\frac{1}{2}$  hour until the bath is exhausted.

b. *Development*.—Prepare a fresh bath containing 1 kg. of sulphocyanide of ammonia and 1.5 kg. of bichromate of potash, treat for  $\frac{1}{4}$  hour at 30° C. and add slowly 10 gr. of sulphuric acid of 66° Bé. per liter of liquor, raise to 85° C. in  $\frac{1}{2}$  hour, treat for  $\frac{1}{2}$  hour at 85–90° C., rinse, neutralize, and 10 rinse thoroughly again.

*Example for silk*

(IV) a. *Dyeing*.—10 kg. of natural, unweighted silk are dyed cold for  $\frac{1}{4}$  hour with 15 20 gr. of estersalt of leuco-2-(5:7-dibromo-indol)-2-anthracene-indigo and an addition of 200 gr. of rongalite C (Colour Index, page 364) and 200 gr. of acetic acid of 80% (dye-liquor=800 liters). After having further 20 added 200 gr. of formic acid of 80%, dye again cold for 10 minutes and raise the temperature during  $\frac{1}{2}$  hour to 80° C., maintain this temperature for  $\frac{1}{2}$  hour and rinse.

b. *Development*.—Prepare the oxidizing 25 bath (800 liters) with 200 gr. of sulphocyanide of ammonia and 60 gr. of bichromate of potash and treat for  $\frac{1}{4}$  hour at 30° C. After having slowly added 4 kg. of sulphuric acid of 66° Bé, heat up in  $\frac{1}{2}$  hour to 80° C., treat 30 for  $\frac{1}{2}$  hour at 80–90° C., rinse, neutralize and soap with 5 gr. of Marseille soap per liter of liquor for  $\frac{1}{4}$  hour near to boiling point.

In these examples the sulphocyanide of ammonia may be replaced by another soluble salt of hydrosulphocyanic acid, for instance by an alkaline salt of the said acid.

The present process may also be applicable for ester-salts derived from insoluble dyestuffs other than vat-dyestuffs. Ester-salts of 40 such a kind may be bodies which—besides the essential quinone groups (reduced and esterified) as mentioned in the introduction—contain for instance azo groups (see German Patent No. 461,500, British Patent No. 45 333,507). It is evident that from such an ester-salt the corresponding insoluble dyestuff can be reformed by acid oxidation.

What I claim is:—

1. A process for dyeing animal fibers with 50 esterlike derivatives (ester-salts) of insoluble dyestuffs, containing quinone groups—the latter being in a reduced form and esterified—by applying said bodies on the fiber and subsequently developing the colour thereon by acid oxidation, said process being characterized by performing this development in the presence of watersoluble salts of hydrosulphocyanic acid, the latter acting as buffer substance.

2. A process for dyeing animal fibers with 60 esterlike derivatives (ester-salts) of insoluble dyestuffs, containing quinone groups—the latter being in a reduced form and esterified—by applying said bodies on the fiber and subsequently developing the colour thereon

by acid oxidation, said process being characterized by adding watersoluble salts of hydrosulphocyanic acid to the acid oxidizing bath.

3. A process for dyeing wool with esterlike 70 derivatives (ester-salts) of insoluble dyestuffs, containing quinone groups—the latter being in a reduced form and esterified—by applying said bodies on the fiber and subsequently developing the colour thereon by 75 acid oxidation, said process being characterized by adding watersoluble salts of hydrosulphocyanic acid to the acid oxidizing bath.

4. A process for dyeing wool with esterlike 80 derivatives (ester-salts) of insoluble dyestuffs, containing quinone groups—the latter being in a reduced form an esterified—by applying said bodies on the fiber and subsequently developing the colour thereon by acid 85 oxidation, said process being characterized by adding sulphocyanide of ammonia to the acid oxidizing bath.

In witness whereof I have hereunto signed my name this 9th day of December, 1930.

SIGISMUND FUCHS.

90

95

100

105

110

115

120

125

130